

1

**3,376,245**  
**ANTISTATIC COMPOSITION CONTAINING**  
**POLYEOPOXIDE RESIN**

Byron A. Sample, Jr., Bertie J. Reuben, and Julian J. Hirshfeld, Decatur, Ala., assignors to Monsanto Company, St. Louis, Mo., a corporation of Delaware  
No Drawing, Filed May 15, 1964, Ser. No. 367,860  
9 Claims. (Cl. 260—29.2)

## ABSTRACT OF THE DISCLOSURE

This invention relates to a novel composition and process of rendering antistatic protection to a synthetic textile without discoloring the same by incorporating phosphoric acid or hypophosphorus acid in an aqueous dispersion of an antistatic composition consisting of a high molecular weight polyamine and a polyepoxide obtained as a condensation product of epichlorohydrin and a polyol.

This invention relates to compounds which, when applied to a synthetic textile fiber, have antistatic characteristics. More particularly, this invention relates to antistatic compounds which when applied to synthetic fibers in the presence of a phosphorus containing acid render an undcolored, static free fiber.

Synthetic fibers when coming into contact with foreign objects tend to collect static electrical charges thereon which is objectionable during the manufacture and wearing thereof. The accumulation of static charges thereon prevents the finished fabrics from draping like cotton or wool and causes the same to cling uncomfortably to the wearer. The static charges also attract dust and lint to the fabric. It is well known in the art that polyamines are effective temporary antistatic agents and when associated with the fibers which comprise a fabric in the presence of a polyepoxide, the polyamine molecules and the polyepoxide molecules crosslink thereon and become durably attached thereto. The methods and compositions are clearly shown in U.S. Patent No. 3,021,232 to Pretka and U.S. Patent No. 2,982,751 to Anthes, respectively. However, it has been found that when a fiber is treated with a polyamine compound, a discoloration results which is undesirable and which lowers the commercial value of the fiber. An afterwash is only partially effective for it does not remove all of the discoloration. It also is an additional operation which is objected to as being time and money consuming. It is to this problem that attention of this application will be directed.

Therefore, an object of this invention is to provide a novel process which will impart to a synthetic textile fabric antistatic properties without discoloring the same.

Another object of this invention is to provide a novel composition of matter which renders antistatic protection to a synthetic textile fabric without discoloring the same.

A further object of this invention is to provide synthetic fibers which retain their original color with an antistatic agent.

A still further object is to provide a water-soluble antistatic composition which is compatible with pH sensitive yarn-finishing ingredients.

These and other objects will become apparent in the course of the following specifications and claims.

In accordance with a preferred embodiment of the present invention, a synthetic textile fiber is provided with durable antistatic properties by continuously associating the fiber, either during the spinning thereof or when the fiber is in fabric form, with an aqueous polyamine/epoxy resin suspension which also contains a third ingredient. This third additive controls the pH of the suspension which is tantamount to controlling the fiber whiteness

2

and the tenacity with which the polyamine clings to the fiber. The polyamine polyepoxide solution readily polymerizes on the synthetic fiber at pH values above 7.0. However, the increase in pH increases the discoloration. Although a decrease in pH prevents to a certain degree the discoloration of the fiber due to the treatment, it decreases, at the same time, the effectiveness of the treatment. This invention discloses the art of reducing the pH for complete prevention of discoloration without any decrease of the effectiveness of the treatment.

The use of these antistatic agents, in accordance with the present invention, effects improvements in the characteristics of acrylonitrile polymers and articles produced therefrom. This invention is applicable not only to polyacrylonitrile, but also to copolymers, interpolymers and blends thereof, particularly those containing at least 80 percent by weight of polymerized or copolymerized acrylonitrile. Such polymeric materials include acrylonitrile fiber-forming polymers with readily dyeable basic copolymers the blend having an overall polymerized acrylonitrile content of at least 80 percent by weight.

An acrylic fiber may be formed by extruding a typical acrylonitrile-based spinning dope through a conventional spinnerette into an aqueous coagulation bath wherein the dope hardens into a filament. After the fibers were washed and stretched as they were drawn up a hot water cascade, they are heated and partially dried on a set of drying rolls. When the moisture content of the fiber is approximately 20 percent by weight and the temperature of the filaments has reached approximately 100° C., they are immersed in an aqueous emulsion which contains

- (a) a polyamine,  
(b) an epoxide resin, and  
(c) a lubricant.

Where the aqueous emulsion is applied to a fabric by padding, or the like, the lubricant may be eliminated for there is no problem of the fibers wrapping around the drying rolls. However, where the antistatic finish is being applied to synthetic fibers during the manufacture thereof, a lubricant is a necessary additive for the fibers have the tendency to stick to the drying and curing rolls without it. The mixture preferably contains a dispersing or emulsifying agent which insures a more homogeneous suspension of the several ingredients. The temperatures of the suspension is generally held at below 40° C. in order to prevent premature polymerization.

The use of polyamine compounds as antistatic agents, while being an excellent antistat, is limited to applications where the aqueous emulsion is kept at a pH of below 7. If the pH of the suspension is allowed to rise above 7, the effectiveness of the antistat is destroyed somewhat for the discoloration limits the use of the fiber. Further, the effectiveness of the antistatic finish is reduced as the pH approaches zero. By the addition of phosphorous containing acids to the suspension, the pH can be effectively reduced to the desired level without adversely affecting the antistatic properties of the treatment. The reduction of the pH destroys the discoloring characteristics of the polyamine thereby allowing the polyepoxide/polyamine solution to readily polymerize on the surface of the fibers. It has been found that only the phosphorus containing acids have these characteristics and of these, the most effective ones are phosphoric acid and hypophosphorus acid. Either of these acids are added directly to the polyepoxide/polyamine suspension before the fiber is immersed therein. The acids also aid in the dye receptivity of the fiber.

An example of a polyamine in accordance with the present invention is a polyamine having the formula:



when  $-D-$  is a divalent radical terminating in amino nitrogen,  $-A-$  is a divalent radical selected from the group consisting of



and a mixture of these radicals wherein  $-R-$  is a lower alkyl radical,  $-E-$  is a divalent radical selected from the group of desoxy  $-A-$  radicals (i.e., an  $-A-$  radical without its oxygen atom),  $m$  is a whole number from about 5 to 85 and  $n$  is a whole number from about 1 to about 50. The preparation of these polyamines is discussed in Belgian Patent No. 554,506, granted Jan. 25, 1957.

The epoxide resin referred to above can be prepared by condensing epichlorohydrin with a polyol. A typical example is the condensation product (with elimination of HCl) of glycerine and epichlorohydrin. The preparation thereof is described in detail in British Patent No. 780,288, dated July 31, 1957. Such material is available on the open market under the trademark "Eponite 100."

When an aqueous bath is prepared from water, a polyamine, an epoxy resin, and a reducing agent, it is desirable to add thereto a dispersing agent to insure a thorough mixture of the respective ingredients. Satisfactory dispersing or emulsifying agents are the aromatic polyglycol ethers, one example of such being the alkyl-phenol polyglycol ether containing 9.5 moles of ethylene oxide which can be purchased on the open market under the trademark "Neutronyx 600."

The effectiveness of the phosphorus containing acids in reducing discoloration was checked in the manner as set forth below. Where the antistatic emulsion is applied to a

Chromey apparatus to determine the level of static protection after selected washings. To determine the effectiveness of the phosphorus containing acids in preventing discoloration of the synthetic fibers at lower pH levels, the fabric is tested according to standards established by the American Association of Textile Chemists and Colorists. Such test results are then compared with emulsions which do not contain the phosphorus containing acids. The examples will show that in every test run, the gray scale rating for the treated fabrics increased from an unacceptable value to an acceptable one upon the addition of the phosphorus containing acids.

The following examples are cited to illustrate the invention. They are not intended to limit this invention in any way. Unless otherwise noted, "parts" as expressed in the examples indicate parts by volume.

#### Example I

A sample of acrylic fibers consisting of a copolymer of 93 percent acrylonitrile and 7 percent vinyl acetate in the form of a tow or fabric were treated by padding, dripping, washing and the like, with an aqueous emulsion having the following constituents:

|                  | Percent |
|------------------|---------|
| Polyamine        | 5       |
| Polyepoxide      | .5      |
| Polyglycol ether | .125    |
| Water            | 94.22   |

The total finish solids constituted at least 0.4 percent of the weight of the fiber. The pH of the above aqueous emulsion was adjusted 6.5 by the addition of phosphoric acid. Several tests were run wherein the total finish applied to the fiber was varied over a wide range by changing the relative concentrations of the finish ingredients which comprise the aqueous emulsion. Table I (immediately below) compares the Gray Scale Rating of the emulsion containing and not containing phosphoric acid, the highest on the Gray Scale Rating being 5 and the lowest being 1.

TABLE I

| Suspension                                 | Gray Scale Rating |             |            |              |                  |
|--------------------------------------------|-------------------|-------------|------------|--------------|------------------|
|                                            | pH                | As Received | Blank Dyed | Basic Dyeing | Dispersed Dyeing |
| Polyamine/Polyepoxide                      | 9.9               | 2           | 1-2        | 1            | 1-2              |
| Polyamine/Polyepoxide with Phosphoric acid | 6.5               | 3-4         | 2-3        | 2            | 2-3              |

tow, the finished filaments are converted into yarn and the yarn is knitted into a tubular fabric shape whereupon the fabric is blank dyed by any conventional dyeing process. Where the antistatic emulsion was applied to a finished fabric, it was also blank dyed by a conventional dyeing process. Hereinafter, the testing processes are the same for both types of samples. The fabric is washed in a Kenmore washing machine at 100° F. using 0.5 percent "Tide" detergent for four minutes or alternatively, a 0.3 percent solution of tetra sodium pyrophosphate may be used as the detergent. After the tube is removed from the washing machine, it is centrifuged to remove the excess moisture. The steps of washing the tube in the detergent for four minutes, centrifuging it and drying it in an air atmosphere with a relative humidity of 35 percent at a temperature 72° F. are repeated a selected number of times, whereupon the fabric is run on a Hayeck and

| Suspension                                 | After Blank Dyeing Static "Half Life" in seconds |                     |
|--------------------------------------------|--------------------------------------------------|---------------------|
|                                            | 10 Home Launderings                              | 20 Home Launderings |
| Polyamine/Polyepoxide                      | 2                                                | 5                   |
| Polyamine/Polyepoxide with Phosphoric acid | 3                                                | 4                   |

#### Example II

The finish solution applied to acrylonitrile-based fiber as described in Example I was modified by substituting hypophosphorous acid for phosphoric acid and adjusting the pH of the emulsion therewith to 6.5. The remainder of the elements were added in the proportions of Example I. The samples herein disclosed were evaluated according to the procedure of Example I and yielded the results illustrated in Table II.

TABLE II

| Suspension                                      | Gray Scale Rating |             |            |              |                  |
|-------------------------------------------------|-------------------|-------------|------------|--------------|------------------|
|                                                 | pH                | As Received | Blank Dyed | Basic Dyeing | Dispersed Dyeing |
| Polyamine/Polyepoxide                           | 9.9               | 2           | 1-2        | 1            | 1-2              |
| Polyamine/Polyepoxide with Hypophosphorous acid | 3                 | 2-3         | 2          | 3            | 3                |

| Suspension                                           | After Blank Dyeing Static<br>"Half Life" in seconds |                        |   |
|------------------------------------------------------|-----------------------------------------------------|------------------------|---|
|                                                      | 10 Home<br>Launderings                              | 20 Home<br>Launderings | 5 |
| Polyamine/Polyepoxide                                | 2                                                   | 5                      |   |
| Polyamine/Polyepoxide with Hypo-<br>phosphorous acid | 4                                                   | 8                      |   |

As previously described, a synthetic textile filament in the form of a tow or fabric is treated with an aqueous emulsion comprising the mixture of a polyepoxide and a polyamine, the mixture having the pH thereof adjusted by the addition of phosphorus containing acids. The concentration of the reactants in the suspension may vary widely; however, emulsions containing from about 1 percent to about 30 percent by volume of reactants are generally preferred. Such an emulsion will be able to provide a synthetic fiber with an adequate amount of antistatic protection without having the undesirable discoloration which is generally present when a synthetic fiber is associated with a polyamine. After the fiber has been associated with the antistatic aqueous emulsion, the reactants are cured thereon by raising the temperature thereof to 145° C.

Many different modifications of the invention may be made without departing from the scope and spirit thereof. It is contemplated that variations may be made in the percentages of the compounds used without greatly altering the antistatic characteristics of the fiber; therefore, the applicant does not wish to be bound by the numbers exactly as they appear herein.

We claim:

1. An antistatic composition useful for imparting antistatic properties to a synthetic textile without the discoloration thereof, said composition comprised of

(a) a polyamine having the formula:



wherein D is a divalent radical terminating in amino nitrogen, A is a divalent radical selected from the group consisting of



and a mixture of these radicals wherein R is a lower alkyl radical, E is a divalent radical selected from the group consisting of



m is a whole number from about 5 to about 85 and n is a whole number from about 1 to about 50,

(b) a polyepoxide obtained as a condensation product of epichlorohydrin and a polyol,

(c) a phosphorus containing acid selected from the group consisting of phosphoric acid and hypophosphorous acid, and

(d) a dispersing agent.

2. The composition of claim 1 wherein the polyepoxide is a condensation product of glycerine and epichlorohydrin.

3. The composition of claim 1 wherein the dispersing agent is an aromatic polyglycol ether.

4. The composition of claim 1 wherein said composition is comprised of:

(a) about 5.0% of the polyamine,

(b) about 0.5% of the polyepoxide,

(c) about 0.125% of the dispersing agent,

(d) enough of the phosphorus containing acid to adjust the pH of the composition to about 6.5, and

(e) the residue water, the percents based on weight of the composition.

5. A process of imparting antistatic properties to a synthetic textile by treating said textile with the composition of claim 1.

6. The process of claim 5 wherein the synthetic textile is an acrylic textile.

7. A synthetic textile treated by the composition of claim 1.

8. An acrylic filament treated by the composition of claim 1.

9. An acrylic fabric treated by the composition of claim 1.

#### References Cited

#### UNITED STATES PATENTS

2,965,517 12/1960 Albrecht et al. ----- 260—2  
45 3,040,076 6/1962 Seidel et al. ----- 260—615

WILLIAM H. SHORT, Primary Examiner.

T. E. PERTILLA, Assistant Examiner.